

# UNITED STATES PATENT OFFICE.

FREDERICK M. BECKET, OF NIAGARA FALLS, NEW YORK, ASSIGNOR TO ELECTRO METALLURGICAL COMPANY, OF NIAGARA FALLS, NEW YORK, A CORPORATION OF WEST VIRGINIA.

## ZIRCONIUM ALLOY AND PROCESS OF MAKING SAME.

1,425,572.

Specification of Letters Patent. Patented Aug. 15, 1922.

No Drawing.

Application filed October 1, 1920. Serial No. 414,086.

To all whom it may concern:

Be it known that I, FREDERICK M. BECKET, a citizen of the United States, residing at Niagara Falls, in the county of Niagara and State of New York, have invented certain new and useful Improvements in Zirconium Alloys and Processes of Making Same, of which the following is a specification.

This invention relates to a novel alloy consisting essentially of zirconium, silicon and iron, and to a process of making the same.

It is well known that zirconia can be reduced by carbon in the electric furnace, but the resulting product is invariably contaminated by carbon, presumably chemically combined as zirconium carbid. This carbid, in addition to being practically infusible, is only very slightly soluble in molten steel, and the same holds true of high-carbon ferrozirconium. Therefore the direct preparation by carbon reduction of ferrozirconium alloys suitable for use as additions to steel has not heretofore proven practicable.

I have discovered that silicon in sufficient proportion possesses the property of excluding carbon from iron-zirconium alloys, and on the basis of this observation I am able to prepare directly by carbon reduction in the electric furnace, iron-zirconium-silicon alloys which do not contain sufficient carbon to interfere to any material extent either with the electric furnace operation or with the subsequent employment of the alloy in the treatment of steel. Furthermore, the silicon lowers the melting point of the alloy, and increases its solubility or its solution-rate in molten steel.

Following are specific examples in accordance with my invention, it being understood that the invention is not restricted to the particular proportions of charge components mentioned by way of illustration, since these will of course vary according to the specific composition of alloy desired. In all cases, however, the silicon will be in sufficient proportion to the zirconium to exclude any objectionable proportion of carbon from the product; and in the preferred embodiment of the invention the proportion

of silicon will be at least equal to that of the zirconium.

### Example 1.

The charge mixture contained in each 55 2,000 lbs.:

|              |            |
|--------------|------------|
| Silica rock  | 710 lbs.   |
| Zirconia ore | 550 lbs.   |
| Charcoal     | 660 lbs.   |
| Steel scrap  | 80 lbs. 60 |

The zirconia ore used contained:

|                                |         |
|--------------------------------|---------|
| ZrO <sub>2</sub>               | 56.80%  |
| SiO <sub>2</sub>               | 29.67   |
| TiO <sub>2</sub>               | 7.05 65 |
| Al <sub>2</sub> O <sub>3</sub> | 1.64    |
| Fe <sub>2</sub> O <sub>3</sub> | 0.56    |

The alloy produced analyzed as follows:

|    |        |    |
|----|--------|----|
| Zr | 30.33% | 70 |
| Si | 55.34  |    |
| Fe | 11.80  |    |
| Ti | 2.00   |    |
| Al | 0.25   | 75 |
|    | 99.72% |    |

with traces only of carbon.

### Example 2.

The charge mixture contained: 80

|              |            |
|--------------|------------|
| Silica rock  | 830 lbs.   |
| Zirconia ore | 465 lbs.   |
| Charcoal     | 650 lbs.   |
| Steel scrap  | 55 lbs. 85 |

The ore contained:

|                                |         |
|--------------------------------|---------|
| ZrO <sub>2</sub>               | 76.52%  |
| SiO <sub>2</sub>               | 18.08   |
| Fe <sub>2</sub> O <sub>3</sub> | 2.58    |
| TiO <sub>2</sub>               | 0.66 90 |
| Al <sub>2</sub> O <sub>3</sub> | 1.34    |

The alloy produced contained:

|    |            |
|----|------------|
| Zr | 39.32%     |
| Si | 42.68      |
| Fe | 16.54      |
| Ti | 0.46       |
| C  | 0.04       |
|    | 99.04% 100 |

Alloys containing decidedly less zirconium than the foregoing are readily prepared in accordance with this process; but if it be attempted to exceed about 39.5% zirconium content in an alloy containing only 10% of iron, the operation is apt to become erratic, presumably due to the formation of zirconium-carbid. Once this compound has been formed it becomes difficult to remove the

10 product from the crucible, and quite impossible to tap it under ordinary conditions.

Following is an example of the process as applied to alloys of relatively low zirconium content:

15 The charge mixture contained:

|              |           |
|--------------|-----------|
| Silica rock  | 1080 lbs. |
| Zirconia ore | 135 lbs.  |
| Charcoal     | 720 lbs.  |
| Steel scrap  | 65 lbs.   |

20 The ore in this case analyzed:

|                                |        |
|--------------------------------|--------|
| ZrO <sub>2</sub>               | 53.84% |
| SiO <sub>2</sub>               | 28.36  |
| Fe <sub>2</sub> O <sub>3</sub> | 5.12   |
| TiO <sub>2</sub>               | 1.16   |
| Al <sub>2</sub> O <sub>3</sub> | 6.58   |

25 The alloy produced analyzed as follows:

|       |       |
|-------|-------|
| Zr    | 10.0% |
| Si    | 75.0  |
| Fe+Ti | 14.6  |
| C     | 0.1   |
|       | 99.7% |

30 By suitably varying the proportion of steel scrap or equivalent source of iron in the product, low carbon alloys are readily prepared ranging say from 10% or less up to 40% or more of zirconium, together with an equal or greater proportion of silicon, the balance principally iron. It is of course to be understood that other elements, and particularly such as are normal components or impurities of zirconia ores, as for example, titanium, may be present in the alloy in minor proportions without departure from the invention.

My preferred carbonaceous agent is charcoal, although other carbonaceous materials such as coke or coal may be substituted therefor either wholly or in part.

I claim:—

1. A low-carbon ferro-alloy consisting essentially of iron, silicon and zirconium, the silicon and zirconium each in excess of 10%.

2. Alloy according to claim 1 having a zirconium content of 10-40%, the silicon being present in at least as high proportion as the zirconium.

3. A low-carbon ferro-alloy consisting essentially of iron, silicon and zirconium, the silicon content materially exceeding the zirconium content.

4. Process of making a low-carbon ferro-alloy consisting essentially of iron, silicon and zirconium, comprising smelting in the electric furnace a charge comprising silica, a zirconium ore, a carbonaceous reducing agent, and a source of iron, the silica in sufficient proportion to prevent the formation of zirconium-carbid in interfering quantities.

5. Process of making a low-carbon ferro-alloy consisting essentially of iron, silicon and zirconium, comprising smelting in the electric furnace a charge comprising silica, a zirconium ore, a carbonaceous reducing agent, and a source of iron, the charge proportioned to yield an alloy containing silicon in at least as high proportion as the zirconium, whereby the formation of zirconium carbid in interfering quantities is prevented.

6. Process of making a low-carbon ferro-alloy consisting essentially of iron, silicon and zirconium, comprising smelting in the electric furnace a charge comprising silica, a zirconium ore, a carbonaceous reducing agent, and a source of iron, the charge proportioned to yield an alloy containing silicon in material excess of the zirconium, whereby the formation of zirconium carbid in interfering quantities is prevented.

In testimony whereof, I affix my signature.

FREDERICK M. BECKET.